

## UNITED STATES PATENT OFFICE

2,518,710

## LUMAZINES AND ALLOXAZINES AS CATALYSTS IN DYE BLEACH BATHS FOR COLOR PHOTOGRAPHY

Fritz W. H. Mueller, Binghamton, N. Y., assignor to General Aniline &amp; Film Corporation, New York, N. Y., a corporation of Delaware

No Drawing. Application March 27, 1948,  
Serial No. 17,574

8 Claims. (Cl. 95—88)

1

This invention relates to a method of processing photographic color pictures, and particularly to lumazines and alloxazines as accelerators for dye bleach baths used in producing dyestuff images from dyed silver images.

It is known that in the production of photographic dyestuff images from diffusely dyed photographic emulsions containing a silver image, the latter image must be treated with a bleach bath which decolorizes or bleaches the dyestuff present in the photographic layer in the areas where the metallic silver is present. The dyes, which are employed in the diffuse dyeing of the silver-halide emulsion layer, are primarily azo dyes of the substantive and acid type, although some basic vat dyes and alizarines may also be employed. The bleaching or decolorization of the dyestuff is accomplished in a bleach bath in which there occurs a simultaneous decolorization of the dye with an oxidation of the metal image at the points where silver is present, i. e., the metallic silver is converted into a silver compound which may be removed subsequently by fixation in a solution of hypo.

The bleach baths, employed in this process, consist of an aqueous solution of a mineral acid or a mineral acid containing an alkali halide, such as potassium iodide, ammonium chloride, or both. Such baths require a relatively long treating time so as to destroy the dyestuff present in situ with the silver image. Long treatment in bleaching solutions of high acidity has the tendency to soften the gelatin of the photographic emulsion containing a silver image and bleachable azo dye. Moreover, by the use of such baths, a lack of definition of the picture usually follows with other undesirable characteristics. In order to avoid these shortcomings, various organic compounds have been proposed as catalysts which, when added to the bleach bath, accelerate the action of said bath and materially reduce the bleaching time.

The most practical catalysts so far suggested are the azines, such as phenazine, 2,3-diaminophenazine, and the like. Although phenazine and its substituted products are effective as accelerators, they are highly colored substances and are substantive to gelatin, i. e., leave a stain in the gelatin layer which is difficult to remove, and, which seriously affects the quality of the final image.

I have discovered that lumazines and alloxazines, although colored substances ranging from orange to yellowish-green in color, are not substantive to gelatin, do not stain the gelatin layer, 55

2

and do not affect the quality of the final image. The lumazines and alloxazines presumably act as very effective hydrogen carriers becoming readily reduced by the action of the bleach solution with concomitant oxidation of the silver image and destruction of the dye in situ therewith.

The lumazines and alloxazines are characterized by the following general formulae:



and



wherein R and R<sub>1</sub>, which may be alike or different, represent a hydrogen atom, an alkyl or aryl group, e. g., methyl, ethyl, propyl, etc., phenyl, naphthyl, and the like, R<sub>2</sub> and R<sub>3</sub> represent hydrogen or a methyl group, R<sub>2</sub> always being hydrogen when R<sub>3</sub> is methyl and R<sub>3</sub> always being hydrogen when R<sub>2</sub> is methyl, and Z represents the atoms necessary to complete an aromatic or heterocyclic ring, or ring system, e. g., benzene, naphthalene, anthracene, phenanthrene, pyridine, pyrimidine, and the like. The aromatic and heterocyclic rings may be substituted in the various positions by one or more alkyl groups of the same value as R and R<sub>1</sub>, amino, phenyl, sulfanilamido, or fused on a tetrahydrobenzene radical.

The following are examples of the alloxazines employed in accordance with the present invention:

45 (1)



Alloxazine  
Ber. 24, 2364 (1891)  
Ber. 27, 2116 (1894)

|                                                                                      |                                                                                                          |
|--------------------------------------------------------------------------------------|----------------------------------------------------------------------------------------------------------|
| <p>(2)</p> <p><b>3</b></p> <p>7 (or 8)-methylalloxazine<br/>Ber. 32, 1653 (1899)</p> | <p>(10)</p> <p>5</p> <p><b>4</b></p> <p>7,8-tetramethylenealloxazine<br/>Ber. 70, 1302 (1937)</p>        |
| <p>(3)</p> <p>Phenanthrolumazine<br/>Ber. 70, 761 (1937)</p>                         | <p>10 (11)</p> <p>15</p> <p>7,8,9-trimethylalloxazine<br/>Helv. Chim. Acta. 18, 1134 (1935)</p>          |
| <p>(4)</p> <p>Lumazine<br/>Ber. 70, 761 (1937)</p>                                   | <p>20 (12)</p> <p>25</p> <p>6,7-dimethylalloxazine<br/>Ber. 67B, 1442-52 (1934)</p>                      |
| <p>(5)</p> <p>6 (or 7)-methylumazine<br/>Ber. 70, 761 (1937)</p>                     | <p>30 (13)</p> <p>35</p> <p>6,8-dimethylalloxazine<br/>Ber. 67B, 1442-52 (1934)</p>                      |
| <p>(6)</p> <p>6,7-dimethylumazine<br/>Ber. 70, 761 (1937)</p>                        | <p>40 (14)</p> <p>45</p> <p>7-aminoalloxazine<br/>Journ. Indian Chem. Soc. 15, 77 (1938)</p>             |
| <p>(7)</p> <p>6,7-diphenylumazine<br/>Journ. Indian Chem. Soc. 14, 627 (1937)</p>    | <p>50 (15)</p> <p>55 (16)</p> <p>6 (or 7)-phenyllumazine<br/>Journ. Indian Chem. Soc. 14, 627 (1937)</p> |
| <p>(8)</p> <p>7 (or 8)-ethylalloxazine<br/>Helv. Chim. Acta 17, 1516 (1934)</p>      | <p>60</p> <p>65 (16)</p> <p>6,7 (or 8,9)-benzoalloxazine<br/>Ber. 24, 2366 (1891)</p>                    |
| <p>(9)</p> <p>7,8-dimethylalloxazine<br/>Ber. 67, 1826 (1934)</p>                    | <p>70 (17)</p> <p>75</p> <p>Aza-alloxazine<br/>Ber. 71B, 1243 (1938)</p>                                 |

The foregoing lumazines and alloxazines are generally prepared by the condensation of an o-phenylenediamine or its homologues and alloxan.

5 Lumazine is prepared according to the method described in J. Amer. Chem. Soc. 67, 802, (1945) by heating glyoxal bisulfite and 4,5-diamino-2,6-dihydroxypyrimidine together for 5 minutes at a temperature of 90°C.

6 The methyl or phenyl substituted lumazines can be obtained from ketaldehydes, such as methylglyoxal or phenylglyoxal. The di-substituted derivatives can be obtained from diketones, such as diacetyl or benzil.

7 All of the foregoing lumazines and alloxazines can be reduced to form leuco derivatives which can be re-oxidized with considerable ease, a factor which greatly adds to their value as accelerators in accordance with the present invention.

8 The lumazines and alloxazines may be employed in any mineral acid bleach bath, such as, for example, hydrochloric, hydrobromic, hydroiodic or phosphoric acid, with or without the presence of an alkali halide, such as sodium or

9 potassium bromide or iodide, sodium chloride, ammonium chloride, and the like. The concentration of the acid to be employed is dependent upon the character of the gelatin constituting the photographic color emulsion layer or layers.

10 Usually, the concentration of the acid ranges up to 2½ N. I prefer, however, to employ a concentration not higher than normal.

Inasmuch as the lumazines and alloxazines are water-soluble yellow to orange compounds, which do not stain the gelatin, the amount employed as catalyst is not critical. The higher the amount within practical limits the greater the catalytic activity. An amount as small as 0.005 gram per liter of bleach bath shows an appreciable bleaching action in silver bearing images.

11 For practical purposes, amounts ranging from 0.005 to 2.5 grams per liter of bleach bath may be employed. While any one of the lumazines and alloxazines disclosed and contemplated herein may be employed in any mineral acid bleach bath, I prefer, however, to employ the alloxazines shown in Illustrations 1, 2, 4, 5, 8 to 14, and 18 to 24 because of their general availability and ease of preparation.

12 The following examples will illustrate the preparation of a multi-layer color film, in which after exposure, the dye images are obtained by the silver dye bleach process, and the bleach baths containing the alloxazines as accelerators.

#### EXAMPLE 1

13 Three kilograms of a wet gelatino-silver-halide emulsion, containing about 10% gelatin, 4-5% of silver-bromoidide, 10 cc. of a 10% solution of saponin, and 10 grams of diphenyl biguanide hydrochloride, were separated into three equal portions of 1 kilograms each and utilized in the preparation of the final red, green, and blue sensitive emulsions.

14 To the first portion of a red sensitized wet gelatino silver-halide emulsion there were added 5 grams of a bleachable cyan dye, Direct Sky Blue (C. I. #520).

#### Red sensitive

15 To the first portion of a red sensitized wet gelatino silver-halide emulsion there were added 5 grams of a bleachable cyan dye, Direct Sky Blue (C. I. #520).

#### Green sensitive

16 To the second portion of a green sensitized wet gelatino silver-halide emulsion there were added



1.25 grams of a bleachable magenta dye, Fast Acid Magenta B (C. I. #30).

*Blue sensitive*

To the third portion of a blue sensitive wet gelatino silver-halide emulsion there were added an additional 5 grams of diphenyl biguanide hydrochloride as a dye precipitant and 6.8 grams of a bleachable yellow dye, Dianil Yellow 2R (C. I. #650).

*COATING*

The three final silver-halide emulsions, as above prepared, were coated to a dry thickness of approximately 6 microns upon a cellulose acetate film base (or other suitable support such as baryta coated paper) containing an anti-halo coating. The red sensitive silver-halide emulsion was coated first. Over this coating the green sensitive emulsion was coated followed by a coating of approximately 3 microns dry thickness of a yellow filter prepared in accordance with United States Patents 2,036,546; 2,220,187 or 2,390,707. Over the filter layer the blue sensitive emulsion was coated as the outermost layer.

*PROCESSING*

The finished film, prepared in accordance with the foregoing, was exposed and developed for 15 minutes in a black and white developer of the following composition:

|                            |       |     |
|----------------------------|-------|-----|
| Water                      | cc.   | 750 |
| Metol                      | grams | 1.5 |
| Sodium sulfite (anhydrous) | do    | 80  |
| Hydroquinone               | do    | 3   |
| Potassium bromide          | gram  | 0.5 |
| Water to make              | liter | 1   |

Short stopped for 3 minutes in a bath of the following composition:

|                |       |    |
|----------------|-------|----|
| Sodium acetate | grams | 20 |
| Acetic acid    | cc.   | 10 |
| Water to make  | liter | 1  |

Fixed for 3 minutes in a solution of the following composition:

|                                    |       |     |
|------------------------------------|-------|-----|
| Water                              | cc.   | 650 |
| Hypo                               | grams | 240 |
| Sodium sulfite (anhydrous)         | do    | 15  |
| Acetic acid (28% aqueous solution) | cc.   | 45  |
| Potassium alum                     | grams | 15  |
| Water to make                      | liter | 1   |

The fixed film was then cut into 6 equal strips and the strips treated for 10-15 minutes in dye bleach baths of the following compositions:

I (a) Hydrochloric acid, conc cc. 250  
Water to make liter 1

No satisfactory bleaching action on the dyes was observed within 15-30 minutes.

I (b) To I(a) 5 cc. of a 0.1% aqueous solution of riboflavin was added. Appreciable bleaching of the dyes in all silver bearing areas took place.

II (a) Hydrochloric acid, conc cc. 100  
Potassium bromide grams 100  
Water to make liter 1

Slight bleaching action was obtained in 15 minutes in the cyan, magenta and yellow layers.

II (b) To II(a) 0.1 gram of alloxazine was added.

Complete bleach in all layers was obtained within 10-15 minutes with satisfactory color balance.

*EXAMPLE II*

The bleaching treatment of Example I was repeated on the same fixed color film strips, with the exception that lumazine was substituted for alloxazine with similar results.

*EXAMPLE III*

A halogen silver-bearing layer colored with diamine pure blue FF (Schultz Farbslofttabellen 1931, 7th ed. #308) was treated with a bleach solution of the following composition:

|                        |       |      |
|------------------------|-------|------|
| Hydrobromic acid       | cc.   | 250  |
| 7,8-dimethylalloxazine | gram  | .005 |
| Water to make          | liter | 1    |

The dye was completely bleached within 10-15 minutes.

While the present invention has been described in considerable detail with reference to certain preferred procedures, materials and uses, it is understood that the invention is not limited thereto, that numerous variations may be made in the procedures herein described, and that equivalent materials may be substituted. Thus, for example, azo dyes other than those specifically mentioned and utilized in the foregoing examples, may be bleached satisfactorily, provided they are or can be used in the preparation of multi-layer color film in which, after exposure, the dye images are obtained by the silver dye bleach process. Several hundreds of such dyes are known and further reference to them or to their methods of preparation need not be mentioned herein. Accordingly, the scope of the invention is to be defined by the following claims.

I claim:

1. A dye bleach bath for producing a colored image in a photographic emulsion layer containing a bleachable azo dye and a silver image consisting of an aqueous solution of hydrochloric acid, ammonium chloride, potassium iodide and an accelerating amount of an agent selected from the group consisting of lumazines and alloxazines corresponding to the following general formulae:



and



wherein R and R<sub>1</sub> represent a member selected from the class consisting of hydrogen, alkyl and aryl groups, R<sub>2</sub> and R<sub>3</sub> represent a member selected from the class consisting of hydrogen and methyl group, R<sub>2</sub> always being hydrogen when R<sub>3</sub> is methyl and R<sub>2</sub> always being hydrogen when R<sub>2</sub> is methyl; and Z represents the atoms necessary to complete a member selected from the class consisting of aromatic and heterocyclic ring systems.

2. A dye bleach bath according to claim 1 in which the accelerating agent is alloxazine.

3. A dye bleach bath according to claim 1 in which the accelerating agent is lamazine.

4. A dye bleach bath according to claim 1 in which the accelerating agent is 7,8-dimethylalloxazine.

5. The process of producing a colored image in an exposed and developed photographic layer containing a silver image and a bleachable azo dye which comprises bleaching said layer in a bath comprising an aqueous solution of a mineral acid and an accelerating amount of an agent selected from the group consisting of lumazines and alloxazines corresponding to the following general formulae:



and



wherein R and R1 represent a member selected from the class consisting of hydrogen, alkyl and

aryl groups, R2 and R3 represent a member selected from the class consisting of hydrogen and methyl group, R2 always being hydrogen when R3 is methyl and R3 always being hydrogen when R2 is methyl, and Z represents the atoms necessary to complete a member selected from the class consisting of aromatic and heterocyclic ring systems.

6. The process according to claim 5 in which the accelerating agent is alloxazine.

7. The process according to claim 5 in which the accelerating agent is lumazine.

8. The process according to claim 5 in which the accelerating agent is 7,8-dimethylalloxazine.

FRITZ W. H. MUELLER.

#### REFERENCES CITED

The following references are of record in the file of this patent:

| UNITED STATES PATENTS |                 |               |
|-----------------------|-----------------|---------------|
| Number                | Name            | Date          |
| 1,758,752             | Lierg           | May 13, 1930  |
| 2,145,960             | Wheatley et al. | Feb. 7, 1939  |
| 25 2,183,395          | Gaspar          | Dec. 12, 1939 |
| 2,221,793             | Gaspar          | Nov. 19, 1940 |
| 2,261,608             | Tishler et al.  | Nov. 4, 1941  |
| 2,270,118             | Gaspar          | Jan. 13, 1942 |
| 2,346,090             | Staeble         | Apr. 4, 1944  |
| 30 2,410,025          | Gaspar          | Oct. 29, 1946 |